

## UNITED STATES PATENT OFFICE

2,185,548

## METHOD OF DESIZING

Stanley I. Garnett, Providence, R. I., assignor to  
 American Cyanamid Company, New York,  
 N. Y., a corporation of Maine

No Drawing. Application July 16, 1938,  
 Serial No. 219,598

4 Claims. (Cl. 8—138)

This invention relates to an improved process of desizing textiles.

In the past, textiles have been desized after weaving by removing the size, usually a carbohydrate, by using an enzyme. This process is open to a number of difficulties. In the first place, the enzymes are expensive. Secondly, the process requires a relatively high temperature and is slow. It has been proposed to obviate some of the disadvantages in the use of enzymes by employing a strong mineral acid such as sulfuric acid or hydrochloric acid. While this procedure involves some reduction in cost, it is attended by a very serious disadvantage; namely, that strong mineral acids tend to tender the cotton and must be used very cautiously or with specially rapid alkali neutralization.

According to the present invention, all of the economies of strong mineral acids are obtained without any of the disadvantages and in addition, an improved product is obtained by using sulfurous acid as a desizing agent. Sulfurous acid is much cheaper than enzymes, it does not tender cotton goods in effective concentration, it involves no risk of injury to workmen as compared to sulfuric acid, produces whiter and softer goods and requires no penetrant. There is also a lower ash content in the goods than when enzymes are used. At the same time, a lower temperature can be used with sulfurous acid which effects savings in steam.

It is a further advantage of the present invention that it can be used in the ordinary processes of treating goods without changing the equipment or procedure in any material way.

While the present invention is especially for desizing cotton piece goods, it may be also used for desizing other fabrics such as rayon, cellulose acetate and mixtures with other textiles, such as wool, linen, silk and the like.

The present invention can be practiced in any suitable equipment as it requires only a vessel capable of resisting the mildly corrosive action of sulfurous acid and provided with means for heating the goods in sulfurous acid solution. Although the invention is in no sense limited to any particular equipment, it is an advantage that the standard equipment may be used. Thus, for example, the desizing may be effected in the quench box of any standard singer by simply providing the box with a connection to a cylinder or other source of sulfur dioxide gas and providing for the necessary temperature maintenance. While it is an advantage of the present invention that the desizing can be effected at from 90° to

100° F. as opposed to 125° F. which is necessary with enzymes, the temperature is in no sense critical and high temperatures may be used but they do not present any advantage which compensates for the additional cost of steam. Sulfurous acid from 0.1% to 1.0% is recommended, but higher or lower concentrations may be used.

The invention will be described in conjunction with the following specific examples which illustrate typical embodiments of the invention. The invention, however, is not limited to the exact details therein set forth.

## Example 1

Cotton goods are passed through a singer of 15 standard design and then into the quench box which is filled with a 0.5% solution of sulfurous acid obtained by bubbling sulfur dioxide gas thereinto, the solution being maintained at 100° F. The goods are preferably run through the 20 quench box open width and then through two pot eyes and over a reel into a box truck or are pulled over into pits and permitted to lie for several hours. The speed is so regulated that a time of impregnation of from 0.4 to 6.0 seconds results. 25 Normally from 2 to 4 hours is sufficient to effect thorough action of the sulfurous acid on the starch, but it is an advantage of the present invention that the goods can be permitted to stand up to 4 days without injury to the fabric. After 30 thorough action of the sulfurous acid on the size, the goods are then further processed in the normal manner which, with cotton goods, essentially involves kier boiling, followed by washing, souring, bleaching and the like. These further steps 35 do not depart from standard practice and the only difference is that the goods are whiter than would otherwise be the case.

## Example 2

Rayon or cellulose acetate or mixtures with 40 wool, linen, silk and the like are mixed in an aqueous solution of 0.5% sulfurous acid at 100° F. in a 200-gallon box. The goods may be either 45 in open or rope form. The goods are then permitted to lie for 2 hours, washed and boiled off with soap in the usual manner. No injury is noted and goods of exceptional whiteness are produced.

What I claim is:

1. A method for desizing cellulose fabrics sized with a predominantly carbohydrate size which comprises subjecting the fabric to the action of an aqueous solution of sulfur dioxide.
2. A method of desizing cotton goods sized with 55

a predominantly carbohydrate size which comprises singeing the goods, quenching them in an aqueous solution of sulfur dioxide, and permitting the goods to stand for sufficient time to effect action of the sulfurous acid on the size.

3. A method according to claim 1 in which the

desizing is effected at temperatures between 90° and 100° F.

4. A method according to claim 2 in which the desizing is effected at temperatures between 90° and 100° F.

STANLEY I. GARNETT.